

## UNITED STATES PATENT OFFICE

2,191,034

## MANUFACTURE OF GELATIN

Samuel E. Sheppard and James H. Hudson, Rochester, N. Y., assignors to Eastman Kodak Company, Rochester, N. Y., a corporation of New Jersey

No Drawing. Application July 15, 1938,  
Serial No. 219,429

5 Claims. (Cl. 260—118)

This invention relates to a process of producing gelatin for photographic uses.

The gelatin used in photographic emulsions or other photographic layers is subjected, during the processing of the films or plates on which the layers are coated, to alternate alkaline and acid baths. The gelatin must, therefore, withstand changes from high to a low pH and vice versa and, if this change in pH passes through the iso-electric point of the gelatin, there is an alternate swelling and contraction of the gelatin which tends to lower the quality of the photographic image.

In our prior Patent No. 2,101,877, granted December 14, 1937, we described a process of preparing photographic gelatin having an iso-electric point at a higher range on the pH scale, so that the minimum region of colloidal properties, such as swelling in water and change in viscosity in alkaline solution, was higher on the pH scale than in the case of the ordinary gelatin obtained by lime treatment of hides. Our prior process consisted in carrying out the entire hide treatment processes of dehairing and plumping, in an acid solution.

Our investigations have shown that the dehairing of hides for the purpose of producing gelatin from them is most readily and speedily effected in alkaline baths, particularly at a pH of 10 or higher.

It is, therefore, an object of the present invention to provide a method for obtaining a photographic gelatin from animal hides in as convenient and rapid a manner as possible, while at the same time producing gelatin having an iso-electric point in the region of pH 6 to 7 or higher. A further object is to provide a more rapid method for obtaining gelatin from hides. A still further object is to provide a method for preventing swelling of the hide material during the dehairing treatment. Other objects will appear from the following description of our invention.

These objects are accomplished according to our invention and a gelatin of high iso-electric region is produced by carrying out the dehairing operation in an alkaline medium, but with a sufficient concentration of neutral salt present to prevent plumping or swelling of the hide material by the alkaline bath. The subsequent operation of plumping is then carried out in acid medium, as described in our prior Patent No. 2,101,877.

The "iso-electric point" of a gelatin has been defined as the condition at which there is no migration to the anode or the cathode in an elec-

tric field. This condition results from the neutralization of the positive and negative ions in solution. In our prior Patent No. 2,101,877, we referred to the colloidal properties of gelatin, such as swelling in water, change in viscosity in aqueous solution and precipitation from solution by alcohol and grouping these properties together as general physical properties of the gelatin. It is known that, in general, these various physical properties are at a minimum value at the same pH and this minimum of physical values has been taken as an index of the iso-electric point of the gelatin.

The iso-electric point of gelatin depends upon the conditions under which it is extracted from the hides. Gelatin extracted in the usual way by a lime treatment of hides has an iso-electric point at a pH of about 4.7 to 5.1. The gelatin produced by the acid process of our prior Patent No. 2,101,877 has an iso-electric point in the region of pH 7 and upward, and the properties are not nearly so sharply defined at one point as in the case of the lime-processed gelatin. This means that the physical properties, such as swelling, change more gradually with change in pH in the case of the acid-type gelatin.

In the customary alkaline treatment of hides preparatory to extraction of gelatin, the hairs are dislodged and there is a swelling or penetration of the surface or epidermal layer by the alkaline bath. The penetration continues into the hides and it is this treatment which results in the gelatin of low iso-electric point. In the acid treatment described in our Patent No. 2,101,877, there is little swelling of the hide surface. In this case, the individual hairs do not detach themselves from the skin but the whole epidermal layer finally slips, carrying the hair with it. This action is liable to be somewhat unequal especially with the skins of older animals and, for this reason, the treatment is not always satisfactory. This condition can be avoided, however, by restriction of the swelling action of an alkaline bath designed to dehair the skin, to the surface or epidermal layer whereby the action of the alkaline material is limited to a chemical reduction of the keratin of the hair roots, so that the hair slips out easily on slight rubbing. This chemical action is probably the conversion of disulfide linkage in the keratin to two SH groups. This type of dehairing which corresponds to that effected in regular lime baths, except in that plumping of the hide is prevented is, therefore, entirely different from that which occurs in a wholly acid treatment of the hides. If the alkaline treatment

5

10

15

20

25

30

35

40

45

50

55

is carried out in the usual way, it does result in swelling of the hide substance but, by providing a sufficient concentration of neutral salt in the alkaline bath, the plumping or swelling of the hide material is prevented, while, at the same time, allowing the chemical reduction to proceed so that the hairs may be readily removed.

After the dehairing treatment which requires from several days to a week, the hairs may be removed by slight rubbing, such as by washing in a mill. The stock is then removed to an acid plumping bath where it is left for a sufficient length of time for full plumping or swelling to take place. This action may require a week or longer.

After completion of the plumping, the hide pieces are neutralized to a pH of 5 to 7. The acid liquor may first be drained from the stock, or the hide pieces may be neutralized in the acid solution. It will be preferable, of course, to drain the acid liquor from the hide stock so that it is not necessary to neutralize the acid liquor. The progress of the neutralization may be estimated by slicing through a number of pieces of hide selected at random and treating the fresh surfaces in turn with the following indicators to determine the pH:

|                   | pH      |
|-------------------|---------|
| Bromocresol Green | 4.0-5.6 |
| Chlorphenol Red   | 5.2-6.8 |
| Bromthymol Blue   | 6.0-7.6 |

This illustrates the pH range which may be indicated by various compounds. Color nuance may be estimated by these dyes with an accuracy pH of .2 to .4.

When the central portions of the hide have attained the pH desired, the material is subjected to extraction with hot water at a temperature of 160 to 180° F. The pH at which extraction takes place may vary and, although it may be as high as 6 or 7, we have found that a pH of 5 is satisfactory because this is not so acid as to produce excessive hydrolysis of the gelatin while, on the other hand, it is sufficient acid to prevent saponification of fats and, therefore, to allow their ready separation. The gelatin liquor is then filtered and may be vacuum concentrated before chilling and drying.

The following examples which are illustrative only indicate several methods of extracting gelatin, according to the present invention.

#### Example I

A quantity of green calf hide was washed to remove excess salt, dirt and other foreign matter and was then treated with an aqueous solution containing 1% NaOH and 7% Na<sub>2</sub>SO<sub>3</sub>. After twenty-four to seventy-two hours, the hair was found to slip easily from the hide and was removed by washing the stock in a mill. It was then removed by washing the stock in a mill. It was then removed to an acid plumping bath composed of a 1% solution of hydrochloric acid in water. After remaining in the plumping bath for 14 days, the hides were removed and neutralized to a pH of about 5. The gelatin was then extracted from the hides by treating them with hot water at a temperature of 170° F. and the gelatin liquor removed by filtration. The gelatin obtained in this way had a pH of about 5, and an iso-electric point at pH 7 to 9.

#### Example II

A quantity of hide stock was washed to remove foreign matter and was then treated in an

aqueous solution containing 1% NaOH and 1% Na<sub>2</sub>SO<sub>3</sub>. After three days, the hair was removed by washing and the hide was then transferred to a plumping bath consisting of an 0.8% hydrochloric acid solution in water. The hides were allowed to remain in the plumping bath for twenty-one days and, after neutralization, the gelatin was extracted in the usual way and was found to have an iso-electric point at pH of about 6.

#### Example III

A quantity of hides was washed to remove foreign matter and was then subjected to a dehairing bath containing 0.66% NaOH and 6.6% Na<sub>2</sub>SO<sub>3</sub> in water. After six days, the hair was removed by washing and the hides were transferred to a plumping bath. This bath consisted of a 1% acetic acid solution in water and the hides were treated for about fifteen days. They were then removed from the bath and neutralized and the gelatin extracted in hot water in the usual way to produce a gelatin having an iso-electric point at a pH of about 6.8.

#### Example IV

A quantity of greenhide stock was dehaired as described in Example III and was treated in a plumping bath consisting of a 1% hydrochloric acid solution for two days and a 3% hydrochloric acid solution for twelve days immediately thereafter. The hide pieces were then removed from the plumping bath, neutralized, and the gelatin extracted in hot water in the usual way. This produced a gelatin having an iso-electric point at a pH of about 6.7.

The dehairing treatment may be carried out in a solution of any suitable alkaline material, although calcium hydroxide and sodium hydroxide are found to be most suitable. The strength of alkali may vary from 1/4% to about 1% or higher. This bath may contain any neutral inorganic salt, such as sodium sulfite, sodium sulfate, sodium acetate, calcium sulfate, calcium chloride, calcium nitrate, calcium acetate, sodium chloride, sodium nitrate, potassium sulfite, potassium sulfate, potassium chloride, potassium nitrate, and others. The concentration of the neutral salt must be such that swelling of the hide material is prevented, a concentration of from about 1% to about 10% or more of the neutral salt having been found to be satisfactory. The hides may be treated in the dehairing bath for periods varying from about twenty-four hours to about a week.

The plumping treatment of the hides may be carried out as described in our prior Patent No. 2,101,877 in a dilute solution of a weakly ionized acid, for example, a 1/2% to 10% solution of acetic or propionic acid, or in a dilute solution of a strongly ionized acid, such as hydrochloric or sulfuric of a strength of about 0.1% to about 1.0%. The length of plumping treatment may be varied, depending upon the strength of the acid used and the desired pH of the resulting gelatin. Usually a period of from two days to twenty-five days is sufficient for full plumping to take place.

Numerous modifications of our process may be made within the scope of our invention and it is to be understood that we intend to be limited only by the scope of the appended claims.

What we claim is:

1. The method of preparing photographic gelatin having an iso-electric point in the region pH6 to pH9, which comprises subjecting animal hides to a dehairing treatment in a 1/4% to about 1% 75

alkaline solution containing from 1% to 10% of a neutral salt to prevent swelling of the hide material, removing the hides from the dehairing bath and subjecting them to plumping in an acid bath, neutralizing the hides to a pH of about 5 to 7, and extracting the gelatin from them in water solution.

2. The method of preparing photographic gelatin having an iso-electric point in the region pH6 to pH9, which comprises subjecting animal hides to a dehairing treatment in a  $\frac{1}{4}$  to 1% sodium hydroxide solution containing from 1% to 10% of a neutral salt to prevent swelling of the hide material, removing the hides from the dehairing bath and subjecting them to plumping in an acid bath, neutralizing the hides to a pH of about 5 to 7, and extracting the gelatin from them in water solution.

3. The method of preparing photographic gelatin having an iso-electric point in the region pH6 to pH9, which comprises subjecting animal hides to a dehairing treatment in a  $\frac{1}{4}$  to 1% calcium hydroxide solution containing from 1% to 10% of a neutral salt to prevent swelling of the hide material, removing the hides from the dehairing bath and subjecting them to plumping in an acid bath, neutralizing the hides to a pH of about

5 to 7, and extracting the gelatin from them in water solution.

4. The method of preparing photographic gelatin having an iso-electric point in the region pH6 to pH9, which comprises subjecting animal hides to a dehairing treatment in a  $\frac{1}{4}$  to 1% sodium hydroxide solution containing from 1% to 10% of a sodium salt of an inorganic acid to prevent swelling of the hide material, removing the hides from the dehairing bath and subjecting them to plumping in an acid bath, neutralizing the hides to a pH of about 5 to 7, and extracting the gelatin from them in water solution.

5. The method of preparing photographic gelatin having an iso-electric point in the region pH6 to pH9, which comprises subjecting animal hides to a dehairing treatment in a  $\frac{1}{4}$  to 1% calcium hydroxide solution containing from 1% to 10% of a sodium salt of an inorganic acid to prevent swelling of the hide material, removing the hides from the dehairing bath and subjecting them to plumping in an acid bath, neutralizing the hides to a pH of about 5 to 7, and extracting the gelatin from them in water solution.

25

SAMUEL E. SHEPPARD.  
JAMES H. HUDSON.